

Sept. 29, 1931.

R. L. SEABURY

1,824,795

GRANULAR BODY AND METHOD OF MAKING SAME

Filed July 3, 1926



Fig. 1.



Fig. 2.



Fig. 3.



Fig. 4.



Fig. 5. *Ralph L. Seabury* <sup>Inventor</sup>

*By Spencer, Hardman & Fisher*

*Attorney*

## UNITED STATES PATENT OFFICE

RALPH L. SEABURY, OF TOLEDO, OHIO, ASSIGNOR TO DELCO-REMY CORPORATION, OF ANDERSON, INDIANA, A CORPORATION OF DELAWARE

## GRANULAR BODY AND METHOD OF MAKING SAME

Application filed July 3, 1926. Serial No. 120,540.

This invention relates to compressed granular bodies adapted to be used as bearings, electrical conductors, such for instance as electric brushes, and for other purposes, and to a method of making same.

The invention consists broadly in electroplating the granular body, after molding the same into preliminary shape and baking it in such shape, and then compressing the electroplated body in a die under a considerable pressure to re-arrange the internal structure of the body, to force the electroplating into more intimate contact with the particles composing the body and make the plating less porous, and at the same time imparting the exact shape and size desired to the body.

Another advantage resulting from compressing the electroplated body in a die is obtained by the burnishing, smoothing or polishing action which takes place by reason of the frictional engagement of the sides of the body with the die when the body is forced therefrom. Such automatic burnishing of the article saves an extra operation for such purpose, and in the case of an electric brush or other electrical conductor combines with the compressing action to give the article a better electrical contacting surface.

Other and further advantages of the present invention will be apparent from the following description, reference being had to the accompanying drawings, wherein preferred embodiments of the present invention are clearly shown.

In the drawings:

Fig. 1 is a sectional view taken on the line 1—1 of Fig. 2.

Fig. 2 is a sectional view taken on the line 2—2 of Fig. 1 showing the brush in position immediately before being compressed.

Fig. 3 is a sectional view similar to Fig. 1 showing the brush immediately after being compressed.

Fig. 4 shows the finished brush being ejected from the die.

Fig. 5 shows a perspective view of the finished brush.

In the preferred and practical operation of my process in the manufacture of electric brushes, I employ a mixture composed sub-

stantially of 80% powdered or finely cut copper, 12% powdered lead, and 8% powdered graphite. These materials may be of various degrees of fineness, but I find that the best results are obtained by using materials which would pass through a 100 mesh screen. These powders are intimately mixed together and are then compressed under pressure of about 15 tons per square inch in a die or mold, not shown, suitably shaped to form the brush 10 somewhat larger than the final finished size, but a little narrower than the desired final width. By using the proper amount of material in this molding operation, the brush so formed will have a width  $W_1$  and thickness  $T_1$  slightly smaller than the desired final width and thickness but a length  $L_1$  appreciably longer than the final desired length. The brush thus formed is heated to a temperature of about  $750^{\circ}$  C., which causes a metalization or partial coalescence of the particles composing the brush, thereby imparting a distinctly metallic character to the brush, so much so that it can be hammered or deformed by pressure without disrupting its structure, providing the deformation has not been excessive. The heating, however, should not be such as to cause a general fusing together of the material forming the brush.

After the baking operation the brush is electroplated and then subjected to a pressure of about 15 tons per square inch in a die 14, the size of the aperture 12 of the die 14 corresponding with the desired finished width  $W_2$  and thickness  $T_2$  of the brush, the die being deep enough so that the brush may be pressed from the ends. While it is preferable to electroplate the article after baking, these operations may be reversed, if desired. Therefore, where "baking and electroplating" is called for by the claims, either operation may be first.

The ram 16 is provided with a beveled surface 20 so as to provide an inclined surface 22 of the brush 10. The inclined surface 22 of the brush 10 permits the brush to be placed at a slight angle when mounted on the motor as is well known to those skilled in the art.

After the brush has been re-shaped as dis-

55

60

65

70

75

80

85

90

95

100

closed in Fig. 3 ram, 16 moves outwardly from the aperture in the die 14 to the position disclosed in Fig. 4 and the ram 18 may move through the aperture 12, or the die 14 may move to right to the position disclosed in Fig. 4 so as to eject the re-shaped brush 10 from the die 14.

Upon the application of pressure during the repressing or final shaping operation, the material of the brush adjusts itself to the walls of the die 14, causing a more intimate contact of the particles adjacent to the electroplate, and at the same time there is a reduction in the length of the piece. The electroplated coating is also rendered less porous due to the extreme pressure used and to the fact that the repressing causes the piece to be in very tight contact with the walls of the die even after the pressure has been removed.

When the piece is ejected from the mold, which requires an appreciable pressure, due to the tight fitting of one within the other, the copper plating is burnished or polished by its frictional coaction with the die wall and acquires a high metallic luster. The brush is now ready for use, although it is often desirable to grind the end which fits the commutator in order to remove the copper plating at that point.

The manufacture of electric brushes and other electrical conductors in this manner provides a smooth compressed metallic surface therefor, which makes a good electrical connection with holders or devices with which brought into contact and also gives the articles a pleasing and finished appearance.

In the practicing of my method in connection with the manufacture of self-lubricated bearings, I preferably use a composition of copper powder 82%, tin powder 9%, lead powder 3% and graphite powder 6%. These ingredients after being thoroughly mixed are subjected to a pressure of approximately 20 tons per square inch in a mold wherein the material is given an initial shape, which is preferably that of a hollow cylinder. The molded article is then subject to a baking action, the same as described in connection with the manufacture of the electric brush, and after the baking the article is electroplated to give it a surface coating, preferably of copper or brass. This having been done, the article is immersed in lubricating oil, of which it will absorb a very appreciable quantity. The plated and impregnated article is then repressed in a finishing die, preferably using about 20 tons per square inch. The mold for the original forming of the article should be slightly smaller than the outside dimension of the repressing die, while the inside dimension should be slightly larger, thereby permitting the easy entrance of the baked piece into the repressing die. The repressing of the article causes a shortening

and further compression thereof, thereby resulting in an increase of density and hardness, and also causes the metallic plating to be brought into more intimate contact with the particles composing the article and the plating itself is rendered harder and more durable. During the ejection of the piece from the repressing die the plated surface acquires a metallic luster and smoothness. The repressing, after the oil impregnating operation, causes the oil to be more firmly held within the pores of the bearing than when it is treated with oil after the repressing or final shaping operation. This is, no doubt, due to the fact that the repressing operation serves to imprison or partially seal the oil within the pores of the material.

While the oil impregnating step is particularly desirable in connection with the manufacture of bearings, it is sometimes used and desirable in connection with electric brushes and other articles.

When electroplating the inside or the bearing surface of the piece, it is desirable to use a brass plating in order to secure a lower coefficient of friction. The pressing of this plating gives the article a hard, glossy wearing surface which at the same time is sufficiently porous to permit a slight seepage of oil from the body of the bearing through the plated surface. In this way there is secured a good lubricating effect. When made in this manner, the main body of the bearing can be composed of less expensive materials, such as mixtures of graphite and iron powders. A mixture of 90% iron with 10% graphite can be molded and treated similar to the treatment stated above for the copper graphite composition. Such a composition would be sufficiently porous for the absorption of oil while a brass or bronze electroplating on the inside surface would serve as the bearing surface and the lubricant could seep through the thin and somewhat porous plating.

While the form of embodiment of the present invention as herein disclosed, constitutes a preferred form, it is to be understood that other forms might be adopted, all coming within the scope of the claims which follow.

Having thus described my invention, what I claim as new and desire to secure by Letters Patent is:

1. The method of making granular bodies consisting in pressing the material into initial shape in a mold, said initial shape having a smaller cross sectional area than the final shape, baking the initially shaped body at a temperature less than that which will cause fusing thereof, electroplating the baked body, and subsequently re-shaping the body under considerable pressure at both ends, while it is held in a die, to compact the material of the body and of the electroplat-

ing, and to provide a more intimate connection between the two.

2. The method of making a granular electrical conductor, consisting in initially shaping under pressure the materials forming the article, the initial shape having a smaller cross sectional area than the final shape, then baking and electroplating the article, and then subjecting the electroplated article to a compressing and re-shaping pressure in a die to give the article its finished form.

3. The method of providing a granular body with a metallic coating, consisting in forming the body with a smaller cross sectional area than its final form, then electroplating the body and then subjecting it in a die to a compressing pressure at both ends which compacts both the internal structure of the body and the coating, and causing the body to have a frictional ejecting coaction with the die walls to burnish the compacted coating.

In testimony whereof I have hereunto signed my name to this specification.

RALPH L. SEABURY.

25  
30

35

40

45

50

55

60

65